

# United States Patent [19]

Derrick

[11] Patent Number: 5,015,334

[45] Date of Patent: May 14, 1991

[54] COLLOIDAL COMPOSITION AND ITS USE  
IN THE PRODUCTION OF PAPER AND  
PAPERBOARD

[75] Inventor: Arthur P. Derrick, Cronulla,  
Australia

[73] Assignee: Laporte Industries Limited, London,  
United Kingdom

[21] Appl. No.: 410,820

[22] Filed: Sep. 22, 1989

## [30] Foreign Application Priority Data

Dec. 10, 1988 [GB] United Kingdom ..... 8828899

[51] Int. Cl.<sup>5</sup> ..... D21H 21/10

[52] U.S. Cl. ..... 162/168.1; 162/181.6;  
162/181.8; 162/183

[58] Field of Search ..... 162/181.6, 181.8, 183,  
162/168.2, 168.3

## [56] References Cited

### U.S. PATENT DOCUMENTS

2,795,545 6/1957 Gluesenkamp ..... 162/181.8  
2,838,397 6/1958 Gruntfest ..... 162/168.2  
3,052,595 9/1962 Pye ..... 162/181.8  
4,181,567 1/1980 Riddell et al. ..... 162/181.8  
4,210,490 7/1980 Taylor ..... 162/181.8  
4,711,727 12/1987 Matthews et al. ..... 162/181.8

4,749,444 6/1988 Lorz et al. ..... 162/168.3  
4,753,710 6/1988 Langley et al. ..... 162/181.8

### FOREIGN PATENT DOCUMENTS

796289 1/1981 U.S.S.R. ..... 162/181.6  
1052603 11/1983 U.S.S.R. ..... 162/181.8

Primary Examiner—Peter Chin  
Attorney, Agent, or Firm—Kane, Dalsimer, Sullivan,  
Kurucz, Levy, Eisele and Richard

## [57] ABSTRACT

The composition comprises a water dispersible colloidal siliceous material, such as a swelling clay, in intimate association with a low molecular weight water soluble high anionic charge density organic polymer, such as a polyacrylic acid or a polyamine, the ionicity of the siliceous material being significantly modified by the charge on the polymer. The composition may be produced by reacting the siliceous material and the organic polymer in an aqueous phase system at a concentration, for example, of from 5 to 25% by weight of the polymer on swelling clay solids. The composition is suitable for use as a retention/drainage agent in paper or paperboard production, preferably after the addition of a conventional high molecular weight flocculating agent.

15 Claims, No Drawings

COLLOIDAL COMPOSITION AND ITS USE IN  
THE PRODUCTION OF PAPER AND  
PAPERBOARD

BACKGROUND OF THE INVENTION

1. Field of the Invention

This invention relates to colloidal siliceous composition and to its use in a process for the production of paper and paperboard.

2. Brief Description of the Prior Art

Conventional paper or paperboard manufacture involves forming a fibrous stock containing additives such as pigments, fillers and sizing agents and dewatering the stock on a metal or fabric wire to form the basis for the paper or board sheet. Such processes have been subject to the conflicting requirements that ready drainage of the stock should occur and that there should not be undue loss of additives and of fibre from the stock in the course of drainage, that is, that the retention of such additives and fibre on the wire should be high. This acts not only to give a saving in raw material costs and a reduction in the energy required to dry the sheet but also reduces effluent treatment requirements as a result of a lower content of suspended solids, and lower COD and BOD loadings, in the purge water. Sheet formation and surface properties may also be improved. There have been many attempts to optimise drainage and retention properties by the use of combinations of additives, which include polyelectrolytes such as high molecular weight polyacrylamide and its copolymers, which act as flocculating agents.

It has been proposed to use colloidal swelling clays in conjunction with the high molecular weight, relatively low charge density polyacrylamides which have traditionally been used as flocculants, which may be non-ionic, anionic or cationic in nature and may be selected to suit the charge demand of the stock.

U.S. Pat. No. 3052595, for example, discloses the addition of bentonite to filled stock followed by an acrylamide homopolymer or copolymer which may include at most about 15% by weight of a functional comonomer which may be anionic or cationic in nature, corresponding to a charge density of at most about 2 m.eq./g. The effect of the above combination is that the polymer and the bentonite "are mutually activating whereby increased retention of the filler in the paper web and decreased turbidity of the resulting white water are obtained".

More recently, European Patent Specification No. 0017353 disclosed that the fibre retention and dewatering properties of substantially filler-free stocks may be improved dramatically by including in the stock a high molecular weight; e.g. a molecular weight essentially above 100,000, normally above 500,000 and generally about or above 1 million; polyacrylamide and a bentonite-type clay. The polyacrylamide may contain not more than 10% of either cationic or anionic units and is limited thereby to low charge density material.

This line of development has hitherto culminated in the process described in European Patent Specification No. 0235893 comprising adding a high molecular weight linear cationic polymer to thin stock in a quantity which is greater than that conventionally used to form large flocs, subjecting the flocculated suspension to significant shear and adding bentonite to the sheared suspension. It is explained that the effect of shearing is

to break the flocs down into microflocs which are sufficiently stable to resist further degradation.

SUMMARY OF THE INVENTION

5 The present invention relates to paper and paperboard making processes in which the drainage and retention properties of the stock are modified by the use of an inorganic colloidal material, such as a swelling bentonite or other swelling clay, the colloidal material 10 being of modified ionicity.

DETAILED DESCRIPTION OF THE  
PREFERRED EMBODIMENTS OF THE  
INVENTION

15 The invention may be employed in any paper-making process although one possible application of the invention is to the process described in European Patent Specification 0235893 or modifications thereof in which application improvements in retention and drainage properties have been demonstrated. Another example of a process involving the use of clays to which the present invention may be applied is that described in Finnish Patent No. 67736 which utilises a retention aid comprising a combination of a cationic polymer and an anionic material which may be a bentonite.

20 The modified colloidal material utilised according to this invention is a new composition capable of use even outside the papermaking industry in the many and diverse applications of swelling clays and like colloidal materials.

25 The modified colloidal material according to this invention comprises colloidal siliceous particles, for example of a swelling clay, characterised in that the 30 ionicity of the colloidal particles is modified by intimate association with a low molecular weight water-soluble high charge density polymer.

35 The colloidal siliceous particles envisaged according to the invention comprise layered or three dimensional materials based on  $\text{SiO}_4$  tetrahedra the layered materials being optionally interlayered with other materials such as alumina and/or magnesia octahedra. Layered materials particularly useful in the practice of this invention are the smectite family of clay minerals which are three-layer minerals containing a central layer of alumina or magnesia octahedra sandwiched between two layers of silica tetrahedra and have an idealised formula based on that of pyrophyllite which has been modified by the replacement of some of the  $\text{Al}^{+3}$ ,  $\text{Si}^{+4}$ , or  $\text{Mg}^{+2}$  by cations of lower valency to give an overall anionic lattice charge. The smectite group of minerals includes montmorillonite; which includes sodium bentonite; beidellite, nontronite, saponite and hectorite. Such minerals preferably have a cation exchange capacity of from 80 to 150 m.eq./100 g dry mineral. For use according to the present invention the smectite minerals are preferably in the sodium or lithium form, which may occur naturally, but is more frequently obtained by cation exchange of naturally occurring alkaline earth clays, or

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9

Laporte Industries Limited under the trade name LAPONITE.

In relation to these materials the term colloidal is used to indicate the ability to disperse, or be dispersed, in an aqueous medium to give a colloidal dispersion. Compositions according to the invention, however, need not be in the dispersed state and may, for example, be in a solid particulate form which may be dispersed into the colloidal state at or near the point of use. The size of colloidal-dispersible particles is generally in the range 5  $\times$  10<sup>-7</sup> cm to 250  $\times$  10<sup>-7</sup> cm.

The low molecular weight water-soluble high charge density polymers utilised according to this invention have some or all of the following characteristics which contribute to their effectiveness.

- (a) they are substantially linear, that is they contain no cross-linking chains or sufficiently few not to inhibit water-solubility,
- (b) they are either homopolymers of charged units or are copolymers containing more than 50%, preferably more than 75% and particularly preferably more than 85% of charged units,
- (c) they are of sufficiently low molecular weight to have water solubility. Preferably they have molecular weights below 100,000, but particularly preferably below 50,000 for example, particularly suitably, from 1000 to 10,000, as determined by Intrinsic Viscosity measurements or by Gel Permeation Chromatography techniques. They can preferably form aqueous solutions of at least 20% w/w concentration at ambient temperatures,
- (d) they have a high charge density, i.e. of at least 4 preferably of at least 7 and up to 24 m.eq/g. Particularly preferably the charge density is at least 8 and, for example up to 18 m.eq/g. The charge densities of anionic polymers may be determined by a modification of the method described by D. Horn in Progress in Colloid and Polymer Science Vol. 65, 1978, pages 251-264 in which the polymer is titrated with DADMAC, a cationic polymer identified hereafter, to excess and then back-titrated with polyvinyl sulphonic acid. The same method, unmodified, may be used to determine the charge densities of cationic polymers.

Such polymers are not flocculants and would not normally be considered for use in paper-making processes.

Examples of anionic high charge density water-soluble polymers suitable for use herein are

polyacrylic acid  
polymethacrylic acid  
polymaleic acid  
polyvinyl sulphonic acids  
polyhydroxy carboxylic acids  
polyaldehyde carboxylic acids  
alkyl acrylate/acrylic acid copolymers  
acrylamide/acrylic acid copolymers  
and salts, for example alkali metal or ammonium salts of any of the above.

Examples of suitable cationic high charge density water-soluble polymers are

polyethyleneimines  
polyamidoamines  
polyvinylamines  
polydiallyl ammonium compounds.

The intimate association between the colloidal siliceous particles and the high charge density polymer which is required according to the present invention

may be achieved by a variety of methods. One such method is dry mixing to provide a product which may be transported readily and dispersed in water on site. Alternatively, a dispersion may be produced by the addition of the colloidal siliceous particles to water containing the high charge density polymer. A concentrated dispersion of the modified colloidal siliceous particles according to this invention may be formed by the above methods for ready dilution for addition to paper stock, or may even be added directly to paper stock. Such concentrated dispersions, suitably but not essentially containing a surfactant and preservative and having a concentration based on the dry weight of the siliceous material of at least 50 g/litre but up to the maximum concentration which is pumpable and preferably above 100 g/l and up to for example 250 g/l, are particularly advantageous embodiments of the present invention.

An alternative method of carrying out the invention is to add the colloidal siliceous material and the water-soluble high charge density polymer species successively, in either order of preference, directly to the stock or to a portion of the stock which has been withdrawn temporarily from the process. Successive addition implies that there should preferably be no significant shear, significant stock dilution, e.g. by more than about 20%, or addition of flocculant, between the addition of the siliceous particles and the high charge density polymers. This may be a less efficient embodiment of the invention since the large volume of water present may delay or prevent, to an extent, the association of those species.

It has been found that the colloidal siliceous particles and the water soluble high charge density polymer interact to form composite colloidal species even when, as is preferred, the high charge density polymer is anionic and the colloidal siliceous particles are swelling clay particles based on an anionic lattice by virtue of substitutions in the octahedral layers. The nature of the interaction is not known but may be due to hydrogen bonding involving hydroxyl ions on the clay lattice. The examination of the composite colloidal particles according to the invention by electrophoretic techniques, for example as described below, shows that the siliceous particles and the polymer molecules exist as a single entity in aqueous dispersion and move only as a single species through the electrophoretic cell and, further, that the ionicity of the siliceous particles has been modified by that of the polymer as shown by an alteration in the velocity of the composite particles from that of unmodified particles of the siliceous material.

In the following tests for electrophoretic mobility particles were timed for 5 graticule spacings. The timing distance over 5 graticules was 0.25 mm. The electrode data was:

|                               |                       |
|-------------------------------|-----------------------|
| Applied Potential (V) =       | 90 V                  |
| Interelectrode Distance (l) = | 75 mm                 |
| Applied Field (E) =           | 1250 VM <sup>-1</sup> |

The samples to be tested were prepared as follows. A sodium-form swelling montmorillonite (FULGEL 100) was washed and dried and samples were slurred at a concentration of 1 g/l in demineralised water and, separately, in 0.01 molar sodium chloride solution each at the natural pH of 9.8 and 9.6 respectively. The sodium

chloride addition was to simulate the ionic content of a paper stock. Additionally, a similar slurry in 0.01 molar sodium chloride but adjusted with ammonium chloride to a pH of 7.0 to simulate conditions in a neutral paper stock was prepared. The procedure was repeated using the same clay which had been modified by reaction according to the invention with an anionic water soluble polymer comprising a neutralised polyacrylic acid having a charge density of 13.7 m.eq./g and a molecular weight of 2500 at a loading of 10% by weight of the clay.

The electrophoretic mobilities of these six samples, in every instance towards the positive electrode, was as follows (units  $\times 10^{-8} = M_2 S^{-1} V^{-1}$ ).

|                     | Clay | Clay/anionic polymer | % increase |
|---------------------|------|----------------------|------------|
| pH 9.8 Demin. water | 3.67 | 5.10                 | 39         |
| 9.6 NaCl            | 2.52 | 3.59                 | 56         |
| pH 7 NaCl           | 2.30 | 3.84                 | 67         |

Thus, in the case of an anionic swelling clay and an organic polymer, for example, the natural lattice charge may be increased by, for example, up to about 70%, the amount of the increase being determinable by the charge density of the polymer and the quantity of polymer, but being preferably at least 10%, particularly preferably at least 20%. Similarly, it is envisaged that a charge could be given to a siliceous material having a nett nil charge such as silica.

In a further series of tests conducted under the same conditions the electrophoretic mobility was determined of the same swelling clay which had been reacted according to the invention with the low molecular weight cationic polymer polydiallyldimethyl ammonium chloride having a charge density of 6 m.eq./g. In every instance the composite clay/polymer particles moved towards the negative electrode with the electrophoretic mobilities, in the same units, set out below.

| pH | Medium         | Mobility |
|----|----------------|----------|
| 10 | Demin. water   | 2.89     |
| 7  | "              | 2.00     |
| 4  | "              | 1.62     |
| 10 | .01 molar NaCl | 3.69     |
| 7  | "              | 3.24     |
| 4  | "              | 2.75     |

Preferably the polymer is used in from 0.5% to 25% on the dry weight of the siliceous material, particularly preferably from 2% to 10% on the same basis.

In the application of the present invention to paper-making processes the modified colloidal material of the invention is preferably incorporated with the thin stock prior, for example from 1 to 20 seconds prior, to its entry to the headbox or machine vats. The level of addition may be that usual in the art for swelling clays for example from 0.05% to 2.5% by weight of the siliceous material based on the weight of the furnish solids but may be optimised by conducting standard retention and drainage tests on the treated stock. Excessive addition can result in peptisation and partial dispersion of the preflocculated stock with resulting fall-off of retention and drainage properties.

The invention may be utilised in acid or neutral paper-making systems following on the normal application of high molecular weight cationic flocculants in which systems anionically modified material according

to the invention are preferably utilised. Cationically modified material according to the invention may suitably be utilised in alkaline paper-making systems e.g. those using calcium carbonate filler and operating at a pH of around 8. The invention is applicable however to a wide range of paper-making processes and stocks including those for the production of writing and printing papers, bond and bank grades, newsprint, liner board, security and computer paper, photocopy paper, sack paper, filler board, white lined carbon, wrapping/packaging paper, plasterboard, box board, corrugated board, towelling and tissue papers.

Other additives usually used in the manufacture of paper or paperboard are compatible with the present invention. Among such additives are fillers, clays (non-swelling), pigments such as titanium dioxide, precipitated/ground calcite, gypsum, sizes such as rosin/alum or synthetic sizes such as the alkylketene dimers or alkyl succinic anhydrides, wet or dry strength resins, dyes, optical brighteners and slimicides.

The present invention will now be illustrated by reference to the following tests in which the performance of the present invention was compared with the conventional use of polymeric flocculants and with the process described in European Patent Specification No. 0235893 in which specification a flocculated suspension is subjected to shear and the sheared suspension was treated with bentonite. It is noted that, apart from the improvement in retention and drainage documented in the following tests, a further advantage of the present invention is the capability of giving excellent results even when the flocculated suspension is not subjected to the significant shear stage deemed to be essential according to European Patent Specification No. 0235893.

Britt Jar testing procedures for measuring fines retention (TAPPI Method T.261, 1980) and drainage tests using Schopper Riegler equipment were used. A standard volume of stock was introduced into a standard Britt Jar apparatus and a cationic high molecular weight polymeric flocculant was added in a given quantity followed either by gentle (500 rpm) mixing or by shear mixing (1500 rpm) for 30 seconds. After the slow mixing no reduction of floc size, i.e. shear of the flocs, was observed in any of the tests reported in this specification. After this mixing stage in some tests a given quantity of a commercial swelling clay was added in the form of a concentrated dispersion in water. In some further tests a polymer modified clay according to the invention was added as a preformed dispersion. The modified clay was produced by combining the swelling clay in, for example, the  $H^+$  or  $Na^+$  form with a concentrated solution of the high charge density polymer species at a polymer to clay weight ratio of which could be from about 1% to 20%. For convenience such dispersions were produced in the concentrated form and diluted to a 10 g/l dispersion for addition to the stock. Suitable products according to this invention were also produced by contacting the clay with a concentrated solution of a high charge density polycationic species in high intensity dry mixing equipment. The clay or modified clay were mixed in by gentle 500 rpm mixing for 15 seconds and the retention and/or drainage tests performed to give results expressed as % fines retained by weight of originally present fines and, in the case of the drainage test, as the time in seconds to drain 500 ml of white water from a 1 litre sample of treated stock.

## Tests 1-40

In the following series of tests the cationic polymer flocculant was an acrylamide copolymer with dimethyl aminoethyl acrylate quaternised with methyl chloride and having an acrylamide/aminoethyl acrylate molar ratio of 86/14. It had a charge density of less than 2 m.eq/g and an intrinsic viscosity of 7 decilitres/minute. The swelling clay was a substantially wholly sodium exchanged calcium montmorillonite available from La-  
10 porte Industries Limited as Fulgel 100 (Fulgel is a Trade Name). Where a modified clay was used it was produced by dispersing the clay in a concentrated solution of a high charge density anionic polymer and diluting to 10 g/l concentration as described above. The high charge density polymer was polyacrylic acid having a molecular weight of about 5000 and an anionic charge density of 13 m.eq/g. The stock used in tests 1 to 15 18 was a bleached fine paper stock containing softwood Kraft and hardwood Kraft stocks in a 25/75 weight ratio and a clay filler in about 15%, sized with a cationic rosin emulsion (2% on fibre) followed by alum. The stock was reconstituted by mixing 2.521 thick stock (consistency 5.33, pH 5.0) with 17.51 white water (pH 4.2) to give a consistency of 0.77%, a pH of 4.4 and a fines fraction of 38.6%. In tests 19-40 a similar but not identical stock having a consistency of 0.77% and a fines fraction of 36.6% was used. In the following Tables the % of the cationic flocculant and of the swelling clay are each based on the weight of the furnish solids while the % of the anionic polymer in the modified clay is based on the dry weight of the clay. In the "Shear" column the symbol "o" indicates the gentle mixing and the symbol "+" indicates shear mixing. Tests 7-12, 29 to 31, 39 and 40 are according to the present invention.

Tests 32-35 use finely divided Kaolin Clay (KC) or fine ground Vermiculite (V) in place of the Bentonite.

| Test No. | Cationic flocculant (wt % furnish solids) | Clay (wt % furnish solids) | Polymer (wt % clay) | Shear | Fines Retn. (wt %) |
|----------|-------------------------------------------|----------------------------|---------------------|-------|--------------------|
| 1        | 0.05                                      | o                          | 0.1                 | —     | 70.9               |
| 2        | 0.05                                      | o                          | 0.2                 | —     | 75.6               |
| 3        | 0.05                                      | o                          | 0.35                | —     | 75.4               |
| 4        | 0.05                                      | +                          | 0.1                 | —     | 69.9               |
| 5        | 0.05                                      | +                          | 0.2                 | —     | 71.5               |
| 6        | 0.05                                      | +                          | 0.3                 | —     | 76.2               |
| 7        | 0.05                                      | o                          | 0.1                 | 10    | 76.0               |
| 8        | 0.05                                      | o                          | 0.2                 | 10    | 78.2               |
| 9        | 0.05                                      | o                          | 0.3                 | 10    | 79.2               |
| 10       | 0.05                                      | +                          | 0.1                 | 10    | 79.2               |
| 11       | 0.05                                      | +                          | 0.2                 | 10    | 81.4               |
| 12       | 0.05                                      | +                          | 0.3                 | 10    | 75.2               |
| 13       | 0.05                                      | o                          | —                   | 0.01" | 67.7               |
| 14       | 0.05                                      | o                          | —                   | 0.03" | 65.5               |
| 15       | 0.05                                      | o                          | —                   | 0.05" | 60.8               |
| 16       | 0.05                                      | +                          | —                   | 0.01" | 62.2               |
| 17       | 0.05                                      | +                          | —                   | 0.03" | 58.5               |
| 18       | 0.05                                      | +                          | —                   | 0.05" | 67.3               |
| 19       | —                                         | o                          | —                   | —     | 57.3               |
| 20       | 0.05                                      | o                          | —                   | —     | 80.6               |
| 21       | 0.075                                     | o                          | —                   | —     | 80.7               |
| 22       | 0.1                                       | o                          | —                   | —     | 73.3               |
| 23       | 0.05                                      | +                          | —                   | —     | 77.3               |
| 24       | 0.075                                     | +                          | —                   | —     | 68.3               |
| 25       | 0.1                                       | +                          | —                   | —     | 76.2               |
| 26       | 0.5                                       | +                          | 0.3                 | —     | 82.8               |
| 27       | 0.75                                      | +                          | 0.3                 | —     | 79.8               |

8  
-continued

| Test No. | Cationic flocculant (wt % furnish solids) | Clay (wt % furnish solids) | Polymer (wt % clay) | Schopper Riegler (secs) |
|----------|-------------------------------------------|----------------------------|---------------------|-------------------------|
| 28       | 0.1                                       | +                          | 0.3                 | 82.4                    |
| 29       | 0.5                                       | +                          | 0.15                | 87.0                    |
| 30       | 0.70                                      | +                          | 0.15                | 85.9                    |
| 31       | 0.1                                       | +                          | 0.15                | 85.7                    |
| 32       | 0.05                                      | +                          | 0.3 (KC)            | 63.9                    |
| 33       | 0.05                                      | +                          | 0.3 (V)             | 69.3                    |
| 34       | 0.05                                      | +                          | 0.3 (KC)            | 73.4                    |
| 35       | 0.05                                      | +                          | 0.3 (V)             | 71.0                    |
| 36       | —                                         | o                          | —                   | 19.6                    |
| 37       | 0.05                                      | o                          | —                   | 17.5                    |
| 38       | 0.05                                      | o                          | 0.2*                | 15.0                    |
| 39       | 0.05                                      | o                          | 0.2*                | 11.7                    |
| 40       | 0.05                                      | o                          | 0.2*                | 11.5                    |

" = % by weight of the furnish solids.

\* = followed by 30 seconds shear at 1500 rpm.

## Tests 41-48

In the following series of tests using the same procedure as tests 1-40 a 100% recycled waste stock for box board container middles was used. It had been sized with a stearyl ketene dimer at 1% level. In reconstituted form it had a fines fraction of 26%, a consistency of 0.5% and a pH of 7.0. The same cationic flocculant and swelling clay was used as in the previous tests. Tests 45-48 are according to the invention. In Tests 47 and 48 the polyacrylic acid was the same as that previously used and in Tests 45 and 46 sodium polyacrylate having a similar charge density was used.

35

25

30

35

40

45

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

55

60

65

50

-continued

| Test No. | Swelling Clay % wt | Anionic polymer                  | Fines Retn. % |
|----------|--------------------|----------------------------------|---------------|
| 50       | 0.2                | —                                | 81.4          |
| 51       | 0.1                | Na polyacrylate                  | 84.8          |
| 52       | 0.2                | Na polyacrylate                  | 88.2          |
| 53       | 0.1                | Polyacrylic acid                 | 86.2          |
| 54       | 0.2                | Polyacrylic acid                 | 89.0          |
| 55       | 0.1                | Polymaleic acid                  | 83.9          |
| 56       | 0.2                | Polymaleic acid                  | 86.2          |
| 57       | 0.1                | Polyvinyl sulphonic acid         | 84.3          |
| 58       | 0.2                | Polyvinyl sulphonic acid         | 85.8          |
| 59       | 0.1                | Sodium Polyacrylate              | 82.0          |
| 60       | 0.2                | Sodium Polyacrylate (High m. wt) | 83.2          |
| 61       | 0.1                | Poly DADMAC                      | 77.0          |
| 62       | 0.2                | (Cationic)                       | 81.7          |
| 63       | 0.1                | Polymin SK (cationic)            | 76.2          |
| 64       | 0.2                | Polymin SK (cationic)            | 76.5          |

The sodium polyacrylate and the polyacrylic acid were those used in the previous Tests except for those used in Tests 59, 60 which had a molecular weight of about 15 million and a charge density of 10 m.e./g. The molecular weights and the charge densities of the polymaleic acid were 1000 and 16 m.e./g and of the polyvinyl sulphonic acid were 2000 and 13 m.e./g respectively. DADMAC is polydiallyldimethyl ammonium chloride which is cationic as is the Polymin SK (Trade Name) which is a polyamidoamine. The charge densities of these materials was 6 m.e./g and 7 m.e./g respectively.

## Tests 65-68

The following Tests were carried out using different processing regimes in terms of order of addition of the system components. Unless otherwise stated 0.03 of the cationic flocculant was used. The stock was a Newsprint stock comprising 35% Virgin CTMP pulp and 65% deinked waste. The reconstituted Stock had a consistency of 0.33%, a pH of 5.7 and a fines fraction of 70.3%. Test 65 is according to the invention.

## Test No.

65: The cationic flocculant was followed by shear mixing at 1500 rpm for 30 seconds and then 0.2% by weight of the furnish solids of the Fulgel 100 was added followed by gentle mixing at 500 rpm for 15 seconds and then 0.02% by weight of furnish solids of the polyacrylic acid were added again followed by gentle mixing. The % fines retention found was 88.6%.

66: Test 66 was varied by including the Fulgel 100 clay with the cationic flocculant. The % retention found was 83.5.

67: Test 65 was varied by omitting the Fulgel 100 clay. The % retention was 80.0%.

68: Test 65 was varied by adding the Fulgel 100 clay and the polyacrylic acid first, followed by mixing at 500 rpm for 15 seconds and then by the cationic flocculant which was followed by shear mixing at 1500 rpm for 30 seconds. The % fines retention was 59.4.

## Tests 69-76

In a further series of tests a similar stock to that used in Tests 1-40 having a consistency of 0.79% was used.

In every Test, except 69, 0.05% of the same cationic flocculant by weight of the furnish solids was added to the stock followed by gentle mixing (Britt Jar 500 rpm) for 30 and then, in Tests 71-76, 0.2% on the same basis

of a dispersion of swelling clay followed by gentle mixing for 15 seconds. The clays used and the retention and drainage properties of the resulting web are summarised in the following Table. Tests 74-76 are according to the invention and in these tests the H<sup>+</sup> form acid activated clays were added as an aqueous dispersion also containing 10%, by weight of the clay, of the polyacrylic acid used in Tests 1-40. In further experiments in which the same clays were separated from the polyacrylic acid containing dispersion and subjected to analysis it was shown that the polyacrylic acid was substantially all adsorbed on the clay.

Test 69 is a control test on the untreated stock (no cationic flocculant, mixing, or clay addition).

| Test No. | Swelling Clay                        | % Fines Retn. | Schopper Riegler |
|----------|--------------------------------------|---------------|------------------|
| 69       | Control                              | 50.1          | 43               |
| 70       | No swelling clay added               | 71.9          | 32               |
| 71       | Acid activated Wyoming Bentonite     | 79.0          | —                |
| 72       | Acid activated Los Trancos Bentonite | 77.5          | —                |
| 73       | Acid activated Spanish Bentonite     | 78.7          | —                |
| 74       | As Test 71 but using modified clay   | 85.4          | —                |
| 75       | As Test 72 but using modified clay   | 83.0          | —                |
| 76       | As Test 73 but using modified clay   | 83.4          | 29               |

Wyoming bentonite is a naturally occurring substantially homoionic sodium bentonite. Los Trancos and Spanish bentonites were alkaline earth bentonites converted substantially to the hydrogen form by acid activation.

## Tests 77-79

These tests using headbox stock from a fine paper mill were conducted on a full pilot scale using a 92 cm wide (84 cm Deckle) conventional Fourdrinier machine manufactured by Sandy Hill Corp USA. The machine speed for the tests was 15.24 metres/minute and the basis weight was 80-85 gm<sup>2</sup>. The stock used had a fiber furnish of bleached kraft (22% pine, 23% hardwood), broke 30% and transition stock 25% and contained fortified rosin emulsion size (5 kg/tonne), alum (9 kg/tonne), caustic soda (0.5 kg/tonne) and a kaolin clay (non-swelling)/titanium dioxide filler at a loading of 100 kg/tonne. As received, consistency was 0.41%, pH 4.3 and stuff box freeness 365.

Tests 77 and 79 were initial and final blank runs with no further additives to the stock. Test 78 was according to the invention and involved the introduction of 0.3 kg/tonne of a high molecular weight cationic polymer, available from Vining Industries Inc. as PROFLOC 1510 and having a charge density well below 2 m.e./g, immediately after the fan pump (the last point of shear before the headbox) and, at a point immediately before the headbox, at a rate of 1.5 kg/tonne on a solids basis, a 10 g/l concentration dispersion containing a swelling sodium bentonite which had been treated according to the invention at a level of 10% on a dry clay basis with an anionic polymer consisting of neutralised polyacrylic acid having a molecular weight of 2500 and a charge density of 13 m.e./g. There was no addition of shear between the addition of the cationic polymer and the polymer loaded bentonite.

The retention results given by the three tests were as follows:

| Test           | Tray Water             | White Water |
|----------------|------------------------|-------------|
|                | % First Pass Retention |             |
| 77 (Blank)     | 84                     | 84          |
| 78 (Invention) | 95                     | 95          |
| 79 (Blank)     | 85                     | 85          |
|                | % Fines Retention      |             |
| 77 (Blank)     | 61                     | 66          |
| 78 (Invention) | 87                     | 87          |
| 79 (Blank)     | 63                     | 64          |

## Tests 80-82

A further series of tests were also conducted on the above pilot scale Fourdrinier machine using a newsprint furnish from an operating mill. Machine speed was 45.7 meter/minute and the basis weight of produced paper was set at 48 to 49 gsm. As received the Southern pine furnish was as follows: kraft 27.2%, thermomechanical pulp 52.0%, groundwood pulp 20.8%, broke 3.4%. Consistency 1.08%, pH 4.2 and stuff box CSF-92.

Test 80 was a no treatment blank. Test 81 involved the introduction of 0.2 kg/tonne of a high molecular weight cationic polymer available from Vining Industries, Inc. as "ProFloc" 1545, having a charge density well below 2 m.e./g. immediately after the fan pump. Test 82 was as per Test 81 but with the sequential addition of 1.5 kg/tonne of an anionic polymer treated bentonite according to the invention to an injection point immediately prior to the machine headbox.

Typical results for this series of tests were as follows:

| Test                            | % First Pass Retention            |
|---------------------------------|-----------------------------------|
| 80 (Blank)                      | 74                                |
| 81 (Polymer Retention Aid only) | 82                                |
| 82 (Invention)                  | 86                                |
|                                 | % Reduction in White Water Solids |
| 80 (Blank)                      | 0 (Base)                          |
| 81 (Polymer Retention Aid only) | 27.6                              |
| 82 (Invention)                  | 43.4                              |

These dynamic machine examples illustrate that the invention can give good results on a pilot scale despite the lack of shear or mixing other than the limited natural turbulence of the thin stock itself passing to the headbox of the Fourdrinier machine.

I claim:

1. A paper or paperboard pulp or stock containing a composition, which comprises; a retention agent, which comprises;

a water-dispersible colloidal siliceous material comprising a water-swellable clay having a cation exchange of at least 80 m. eq./100 gm and having particles in intimate association with molecules of a water-soluble organic polymer having an anionic charge density of at least 4 m. eq./gm said anionic polymer being present in an amount of from 0.5% to 25% based on the dry weight of the clay.

2. A process for the production of paper or paperboard, which comprises; providing a fibrous stock in which there is incorporated with the thin stock a retention agent comprising a water dispersible colloidal ma-

- 5 terial comprising a water-swellable clay having a cation exchange capacity of at least 80 m eq/100 g. and comprising colloidally dispersible particles which particles are in intimate association with molecules of a water soluble polymer having an anionic charge density of at least 4 m eq/g said anionic polymer being present in an amount of from 0.5% to 25% based on the dry weight of the clay; and forming paper or paperboard therefrom.
- 10 3. A process for the production of paper or paperboard providing a pulp or stock as described in claim 2, and wherein the retention agent comprising the water dispersible colloidal material is introduced into the thin stock prior to the entry of that stock to the head-box or machine vats, and after the thin stock has exited the fan pump; and forming a sheet of paper or paperboard therefrom.
- 15 4. A process as claimed in claim 2 wherein the quantity of the retention agent which is introduced is from 0.5% to 2.5% by weight of the content of the siliceous colloidal material therein based on the dry weight of furnish solids.
- 20 5. A process as claimed in claim 2 wherein the retention agent is introduced into the stock or pulp by adding the colloidal siliceous material and the high charge density water soluble organic polymer successively to the thin stock or pulp with no intervening addition of shear, dilution or addition of flocculent.
- 25 6. A process as claimed in claim 2 wherein there is introduced into the thin stock, prior to the introduction of the retention agent therein, a high molecular weight organic polyelectrolyte having cationic charge density of below 2 m.eq./g.
- 30 7. A process as claimed in claim 2 wherein the water swellable clay is a smectite.
- 35 8. A process as claimed in claim 7 wherein the smectite is in substantially homoionic sodium, lithium or hydrogen form.
- 40 9. A process as claimed in claim 2 wherein the high anionic charge density organic polymer has a molecular weight below 50,000.
- 45 10. A process as claimed in claim 2 wherein the organic polymer has a charge density of from 4 to 24 m.eq./g.
- 50 11. A process as claimed in claim 2 wherein the organic polymer has a charge density of at least 8 m.eq./g.
- 55 12. A process as claimed in claim 2 wherein the organic polymer is selected from the group consisting of polyacrylic or methacrylic acid or alkali metal or ammonium salts thereof, copolymers containing such acids or salts, polymaleic acid, polyvinyl sulphonic acid, polyhydroxy carboxylic acids, polyaldehyde carboxylic acids or alkali metal or ammonium salts thereof.
- 60 13. A process as claimed in claim 2 wherein there is used 0.5% to 20% of the polymer based on the dry weight of the clay.
- 65 14. A process as claimed in claim 2 wherein the clay particles in intimate association with molecules of the high charge density organic polymer show a modified electrophoretic mobility in comparison with the particles of the clay itself.
15. A process as claimed in claim 14 in which the modification of the electrophoretic mobility is by at least 20%.

\* \* \* \* \*